

B. E. CLARK.  
WHEEL FOR ROLLER SKATES.  
APPLICATION FILED FEB. 11, 1913.

1,130,794.

Patented Mar. 9, 1915.

*Fig. 1.*



*Fig. 2.*



*Fig. 3.*



WITNESSES

*J. S. McArthur*  
*F. T. Chapman*

*Burton E. Clark*, INVENTOR

BY

*E. G. Siggers*

ATTORNEY

# UNITED STATES PATENT OFFICE.

BURTON EARL CLARK, OF PITTSBURGH, PENNSYLVANIA.

## WHEEL FOR ROLLER-SKATES.

1,130,794.

Specification of Letters Patent.

Patented Mar. 9, 1915.

Application filed February 11, 1913. Serial No. 747,751.

*To all whom it may concern:*

Be it known that I, BURTON E. CLARK, a citizen of the United States, residing at Pittsburgh, in the county of Allegheny and State of Pennsylvania, have invented a new and useful Wheel for Roller-Skates, of which the following is a specification.

This invention has reference to improvements in wheels for roller skates, and is designed to provide a wheel free from certain objections which have been found inherent in roller skate wheels as heretofore constructed.

Heretofore roller skate wheels have been made of a glue composition, wood, steel, aluminum, or paper fiber. These different materials have been found to be too soft or too expensive, or in the case of metal wheels they have been found to wear off on the floors of skating rinks, necessitating frequent treatment of the floor to keep it clean and prevent ruining the clothing of the skaters in case of a fall. Wood has the further disadvantage of wearing irregularly and also requiring grit on the floor to prevent slipping. Furthermore, all composition wheels heretofore used have proven to be failures. Again, practically all wheels now in use and prior to the present invention require grit of some kind on the skating surface to prevent slipping, there being a number of such grit preparations on the market and quantities of them are sold.

The wheel of the present invention is a composition wheel burned and tempered so hard that no ordinary file or drill will make any impression on it. The composition is capable of being molded and is combined with metal parts in the form of face plates and a hub to produce a wheel capable of being secured to a skate in the usual manner. The wheels of the present invention are extremely hard showing no perceptible effect after long constant service, and, moreover, they are so hard that they will not pick up gum or dirt from a skating rink floor, and as they do not wear off they can be used on a perfectly white surface like a dancing floor and leave no marks.

A further feature of the present invention is that the grain or surface of the wheel is such that it will not slip in use, producing thereby what is known as a non-slip wheel.

The invention will be best understood from a consideration of the following detailed description, taken in connection with the accompanying drawings forming a part

of this specification, with the further understanding that while the drawings show a practical embodiment of the invention the latter is not confined to any strict conformity with the showing of the drawings but may be changed and modified so long as such changes and modifications mark no material departure from the salient features of the invention.

In the drawings: Figure 1 is an elevation of a completed wheel constructed in accordance with the present invention. Fig. 2 is a section on the line 2—2 of Fig. 1. Fig. 3 is an elevation of the composition member of the wheel with the other parts omitted.

In the drawings there is shown a body member 1 in the form of an annulus having a portion of the sides toward the center depressed as shown at 2, so that such portion of the body member or annulus 1 is thinner at the depressed portion than at the outer portion. Extending axially through the annulus is a hub 3 which may conform generally to hubs such as are employed in the wheels of roller skates for the reception of ball bearings and for the passage of the axle or spindle, and as the structure of the hub forms no part of the present invention no detailed description thereof is deemed necessary. It is customary to form the hubs with a central peripheral groove 4 and when the body member or annulus 1 is in place upon the hub the groove 4 serves as a receptacle for a mass 5 of a cementing material such as sulfur, which will adhere with sufficient tenacity to the hub 3 formed of metal and the body member 1 formed of a composition to be described. The wheel is completed by these plates 6 mounted on the hub and bearing against the sides of the annulus 1, being suitably shaped to conform to the depressions 2 and through such last named parts of the face plates there are passed bolts 7 traversing radial grooves 8 through the depressed portions 2 of the annulus 1 and opening into the central portion of the annulus. The face plates are of slightly less diameter than the annulus 1 so that there is presented at the edge of the wheel a tread portion 9 exterior to the outer peripheral edges of the face plates 6.

The annulus or body portion of the roller is composed of porcelain which presents a fine hard close-grained surface highly resistant to wear, not adherent to gum or dirt which may be found upon a skating rink floor, and, furthermore, presenting a sur-

face which will not slip upon nor mar a polished white floor like a dancing floor even when no dust or grit is placed thereon.

Porcelain has given good results, but is

5 more or less brittle and breaks easily. This is avoided in the present invention by adding to the porcelain white silica, such as is employed in the manufacture of white glass. The silica toughens the porcelain so that it 10 is no longer brittle under the conditions of use. Further, by the addition of arsenic the composition becomes so hardened that files and metal drills have practically no impression thereupon.

15 The composition portion of the wheel is molded into shape and burned in the same manner as is usually employed in the production of porcelain articles. The hub is then placed in the center of the body member and sealed therein with melted sulfur, after which the side or face plates which 20 may be made of steel stampings are applied and the parts are clamped together by the bolts 7. For ornamental and protective purposes the metal parts may be nickel plated, as is customary. The wheels are then finished by being placed upon mandrels and ground true by emery wheels or other suitable devices for a like purpose.

25 30 The face plates 6 are proportioned to the body member 1 which constitutes the tread of the wheel, so that the peripheral or tread portion of the body member projects somewhat beyond the peripheries of the face plates and these last-named members serve to prevent chipping of the body member.

The cost of production of the wheel of the present invention is less than that of a wheel of aluminum or fiber.

35 40 The composition employed for the tread of the wheel is porcelain which may be rendered tough by the addition of silica and rendered hard by the addition of arsenic. Such composition is now known in the trade 45 as white glass composition and the proportions of the ingredients which have proven satisfactory, though by no means the only proportions that may be employed, are as follows:

50 For use on wooden floor surfaces:—

|                           |          |
|---------------------------|----------|
| Porcelain                 | 1 pound  |
| Silica                    | 4 ounces |
| Arsenious acid or arsenic | 1 ounce  |

55 For use on cement surfaces:—

|           |          |
|-----------|----------|
| Porcelain | 1 pound  |
| Silica    | 8 ounces |
| Arsenic   | ½ ounce  |

What is claimed is:—

60 1. A wheel for roller skates having a tread portion composed of hardened and tempered porcelain.

2. A wheel for roller skates having a tread portion of porcelain containing additional silica.

3. A wheel for roller skates having a tread portion of porcelain containing arsenic and additional silica.

4. A wheel for roller skates having a 70 tread portion composed of porcelain, a toughening agent and a hardening agent.

5. A wheel for roller skates comprising an annulus of porcelain with a metallic hub secured thereto, and protecting face plates at 75 the sides thereof exterior to the hub and there provided with clamping means connecting said face plates.

6. A wheel for roller skates comprising an annulus of porcelain with a metallic hub 80 secured thereto, protecting face plates at the sides of the annulus and exterior to the hub, and clamping means connecting the face plates together and traversing the porcelain annulus.

85 7. A wheel for roller skates comprising a molded annular body composed of porcelain with transverse slots opening through the inner periphery of the annulus, a hub united to the annulus and traversing the 90 central portion thereof, face plates on opposite sides of the annulus, and securing devices traversing the face plates and the slots in the annulus.

8. A wheel for roller skates comprising 95 an annular porcelain body forming the tread portion of the wheel, and a metallic hub interior to the annulus with an intermediate cementing material adherent to both the metallic hub and the annulus, and metallic face plates for the annulus exterior to the hub and stopping short of the periphery and otherwise smooth wearing surface.

9. A wheel for roller skates having a 100 tread of hard fine-grained baked and tempered porcelain.

10. A wheel for roller skates composed of 105 molded and baked, hardened and tempered porcelain presenting a fine-grained hard and otherwise smooth wearing surfaces.

110 In testimony, that I claim the foregoing as my own, I have hereto affixed my signature in the presence of two witnesses.

BURTON EARL CLARK.

Witnesses:

W. L. DOWNER,

S. J. ROCKERSHOUSEN.